

## UNITED STATES PATENT OFFICE.

WILFRED J. HEATON, OF SPRINGFIELD, OHIO.

## HOT-BOX COMPOUND.

No Drawing.

Application filed January 19, 1924. Serial No. 687,388.

This invention relates to journal box lubrication and more particularly to a compound for a hot box and in preparing one-half pint of the same the following ingredients are employed mixed at a temperature of approximately 80° to 90° F. in about the proportions stated, i. e.,

Per cent.

|    |                                   |        |
|----|-----------------------------------|--------|
| 10 | Elain oil (commercial oleic acid) | 16.5   |
|    | Lard oil                          | 3.5    |
|    | Mineral oil                       | 39.02  |
|    | Potash                            | 3.10   |
|    | Water                             | 37.88  |
| 15 |                                   | 100.00 |

In using the preparation 1 gill of signal oil is added to  $\frac{1}{2}$  pint thereof, or if preferred  $\frac{1}{2}$  pint of the preparation may be 20 added to 1 gill of signal oil. Signal oil is an illuminating oil well known and used extensively upon railroads for filling signal lanterns.

The compound is of a pasty consistency 25 and is particularly well adapted for use as a lubricant to be applied to shaft bearings,

axle journals and to moving machine parts in general. When so used it prevents generation of heat in the contacting surfaces between which it is applied. By stirring the 30 mixture well it becomes essentially an emulsion of non-saponifiable oil and water held together by soap. In using the compound, it is poured over ordinary cotton waste or wool so that the latter becomes saturated 35 therewith. Thus saturated, the cotton or wool is applied to the journal box or other part. If the journal box is hot or on fire, the fire is first extinguished, and the waste saturated by my compound is stuffed into 40 the journal box and when in place therein more of the compound may be poured over it, finding its way to the proper surface by capillary attraction.

What is claimed is:

A hot box compound consisting of signal oil and the reaction products of elain oil 16.5%; lard oil 3.5%; mineral oil 39.02%; potash 3.10% and water 37.88%.

In testimony whereof I affix my signature.

WILFRED J. HEATON.